

W. G. ABBOTT, JR.  
WATERPROOF FIBER SHEET AND INSOLE MADE THEREFROM.  
APPLICATION FILED JULY 23, 1915.

1,263,186.

Patented Apr. 16, 1918.



Investor  
William G. Abbott Jr.  
by Jas. A. Lomachill  
Atty.

# UNITED STATES PATENT OFFICE.

WILLIAM G. ABBOTT, JR., OF WILTON, NEW HAMPSHIRE, ASSIGNOR TO J. SPAULDING & SONS CO., OF ROCHESTER, NEW HAMPSHIRE, A COPARTNERSHIP COMPRISING EMMA C. SPAULDING AND MARION L. SPAULDING, BOTH OF BOSTON, MASSACHUSETTS, ROLAND H. SPAULDING AND HUNTLEY N. SPAULDING, BOTH OF ROCHESTER, NEW HAMPSHIRE, AND LEON C. SPAULDING, OF BUFFALO, NEW YORK.

## WATERPROOF FIBER SHEET AND INSOLE MADE THEREFROM.

1,263,186.

Specification of Letters Patent. Patented Apr. 16, 1918.

Application filed July 23, 1915. Serial No. 41,579.

To all whom it may concern:

Be it known that I, WILLIAM G. ABBOTT, Jr., a citizen of the United States, residing in Wilton, in the county of Hillsborough 5 and State of New Hampshire, have invented an Improvement in Waterproof Fiber Sheets and Insoles Made Therefrom, of which the following description, in connection with the accompanying drawings, is a specification, like characters on the drawings representing like parts.

This invention relates to a sheet or layer of fibrous material of the character known as chemically-treated fiber, and has for its 15 object to improve such sheet so that a superior product is obtained, which is especially adapted among other uses to be employed in the manufacture of boots and shoes and especially welted boots and shoes, as the in- 20 soles thereof.

Chemically-treated fiber sheets are made from a plurality of plies or layers of paper and are rendered pliable by moisture present in the fiber.

Chemically-treated fiber employed by me 25 is a product composed in whole or in part of cotton rags which are treated with suitable chemicals known to the trade to render the same substantially hard, non-stretchable and 30 non-compressible, and the fiber thus treated is then treated with glycerin or other chemical in the presence of water to render the hard fiber pliable or flexible, the glycerin or other chemical incorporated in the fiber act- 35 ing to retain a sufficient quantity of water to insure the pliability desired.

In accordance with the present invention, 40 the pliable fiber sheet is provided with one or more coatings of pyroxylin or like moisture-repelling material having the property of forming an antifriction wearing surface, whereby the fiber sheet retains its pliability for a relatively long time and is provided with a water-repelling and antifriction 45 wearing surface, which especially adapts the fiber sheet for use as an insole for boots and shoes as a satisfactory substitute for leather insoles.

The fiber sheet may and preferably will 50 be coated with pyroxylin by passing the sheet preferably a plurality of times through a bath of pyroxylin. The fiber sheet thus

treated, is particularly serviceable in the manufacture of boots and shoes especially as the insole thereof, for the reason that 55 such insole remains pliable and firm for a relatively long time, owing to the fact that the coating of pyroxylin forms a water-repelling layer, which prevents the escape of moisture from within the fiber and the entrance of external moisture into the fiber; and further because said sheet is provided with a durable, smooth, antifriction wearing surface, which is bonded with the fibers of the insole and increases the strength thereof, 65 and which reduces to a minimum friction and heat created by movement of the foot of the wearer of a shoe provided with such insole, with the result that sweating of the feet is reduced to a minimum and the life 70 of the insole is increased.

Figure 1 represents in plan a pliable hard fiber sheet in the form of an insole provided on its opposite surfaces with coatings or layers of pyroxylin, and

Fig. 2, a section of Fig. 1, on the line 2—2, on an enlarged scale.

Referring to the drawing, *a* represents a sheet of chemically treated or pliable hard fiber of the character referred to, in the form 80 of an insole, which is provided on its outer surfaces with layers or coatings, indicated by the heavy lines *b*. The interior body portion *d* represents the natural condition 85 of the pliable fiber sheet.

By reference to the drawing, it will be observed that the moisture in the interior portion of the fiber sheet or insole *a*, is practically sealed within the sheet, and that external moisture is also sealed outside of the 90 sheet, consequently the pliability of the insole or of a larger sheet from which the insole *a* is cut will remain unimpaired for a relatively long time under adverse conditions.

It is preferred to use pyroxylin as the surface layer or coating, but it is not desired to limit the invention in this respect, as other varnish materials, such as cellulose acetate, celluloid, resins, thickened oils, asphaltum, 100 etc., may be used.

It will therefore be seen, that a pliable fiber sheet, of either pliable hard or chemically treated fiber when provided with a sur-

face coating of pyroxylin is especially adapted for use as insoles for boots and shoes, as insoles made from such sheet are superior to those made from untreated chemically-treated fiber sheets, in that they retain their pliability and firmness for a relatively long time, are rendered moisture-repellent, are of increased strength, their life is prolonged, and they have the property of reducing friction.

Claims:

1. A sheet of chemically-treated fiber of that character which has within it a medium for rendering the sheet pliable, said sheet being provided at its surface with a layer of pyroxylin which serves to retain said me-

dium within the sheet, repels external moisture and forms an antifriction wearing surface for the said sheet.

2. An insole for boots and shoes composed of a sheet of chemically-treated fiber of that character which has within it a medium for rendering said sheet pliable, said sheet having at its surfaces layers of material which serve to retain said medium within said sheet, repel external moisture and provide the insole with antifriction wearing surfaces.

In testimony whereof, I have signed my name to this specification.

WILLIAM G. ABBOTT, JR.